

Patented Feb. 8, 1927.

1,616,849

# UNITED STATES PATENT OFFICE.

RAPHAEL STUART FLEMING, OF SYRACUSE, NEW YORK, ASSIGNOR TO MERRELL-SOULE COMPANY, OF SYRACUSE, NEW YORK, A CORPORATION OF NEW YORK.

## MOISTUREPROOF ARTICLE.

No Drawing.

Application filed January 4, 1922. Serial No. 526,992.

This invention relates to a moisture-proof paper and a moisture proofing composition for paper, cloth, wood, etc.

As illustrative, paper has been commonly 5 coated on one or both sides, or impregnated with paraffine with the idea of making the same moisture impervious.

A paraffine coating is comparatively stiff and brittle and cools with a rough, flaky surface, and suggests a crystalline structure. 10 A slight bend cracks the coating and permits the passage of moisture in the air even tho the coating may remain impervious to water.

15 Distinction may, therefore, be made between a material which is moisture proof against water, but is not moisture proof against moisture in the air, the latter being in a gaseous or vaporized state as distinguished from a liquid state.

Repeated tests have proven conclusively 20 that paraffine paper even when slightly bent permits passage of moisture in the air and folding of the paper permits the passage of 25 a relatively large quantity of such moisture, so that the paper is not highly effective for the purpose designed.

It is quite necessary in practical commercial use that paraffine paper when used 30 as bags or wrappers should be bent and folded to fit the barrel or other container in which the material is to be shipped, or must be bent or folded to fit the substance to be wrapped, and such bending and folding 35 renders the paper ineffective to prevent the passage of all of the moisture of the air.

It is, therefore, desirable to produce a 40 paper that is substantially completely moisture-proof, not only as against liquid but as against the moisture in the air, and I have produced a bag, wrapper, or coated 45 paper that is practically completely impervious to water, whether in liquid or gaseous state, and I have discovered and produced a saturating material which when applied to paper effects that result.

The paper so produced is comparatively flexible and may be bent and folded without cracking the saturating material, and thereby permitting the passage of moisture whether liquid or gaseous.

The material may be less dense or more liquid than melted paraffine, and seems therefore, to have a greater penetrating capacity.

The base of this coating composition is paraffin and with a suitable quantity of paraffin, I mix preferably a quantity of a grease, as for instance petrolatum, for illustration, 60 as sold under the trade-mark "Vaseline" or a mineral, animal or vegetable oil may be substituted for the grease, for illustration, paraffin oil, lard oil or cottonseed oil.

However, I at present prefer and find most efficient the substance petrolatum, and therefore, I will specifically indicate an embodiment of my invention, in connection with that substance.

70 Preferably with eight parts of paraffin I mix three parts of petrolatum, and when paper is saturated with the composition so formed, it is substantially completely moisture-impervious as against moisture in the air as well as water.

75 The bag, paper, carton or other article or substance to be saturated should preferably be dipped in a body of the composition in liquid form as by that method a complete saturation with application of the composition to both sides of the article or material is effected. It is quite essential to my invention that the composition be so applied as to effect a substantially complete saturation 80 of the article or material with the composition and so that the composition fills all of the interstices of the material and renders the same proof against the passage of vapor thru it.

85 The bag, wrapper, paper or other material so saturated may be utilized for any purpose where it is desired to prevent passage of moisture, and is particularly useful for enclosing food products for the reason that the

treating composition is practically odorless and tasteless and has no material effect upon the enclosed product while maintaining the same in its initial condition of moisture content.

As paraffin and petrolatum are both derived from crude petroleum, the coating material I have described could be made directly from petroleum.

**I claim:**

A moisture-proof article in the form of a bag formed of paper saturated with a composition comprising approximately eight parts of paraffin to three parts of petrolatum.

In witness whereof I have hereunto set my hand this 22nd day of December, 1921.

**RAPHAEL STUART FLEMING.**